

# UNITED STATES PATENT OFFICE.

STEWART J. CARROLL, OF ROCHESTER, NEW YORK, ASSIGNOR TO EASTMAN KODAK COMPANY, OF ROCHESTER, NEW YORK, A CORPORATION OF NEW YORK.

## CELLULOSE-NITRATE COMPOSITION AND PROCESS OF MAKING THE SAME.

1,354,725.

Specification of Letters Patent.

Patented Oct. 5, 1920.

No Drawing.

Application filed January 2, 1920. Serial No. 349,052.

To all whom it may concern:

Be it known that I, STEWART J. CARROLL, a citizen of the United States of America, residing at Rochester, in the county of 5 Monroe and State of New York, have invented certain new and useful Improvements in Cellulose - Nitrate Compositions and Processes of Making the Same, of which the following is a full, clear, and exact 10 specification.

This invention relates to a new cellulose nitrate composition and process of making the same, in which a cellulose nitrate compound is combined or mixed with other substances, so that the resulting product can be advantageously used in the plastic and analogous arts, such, for instance, as sheet or film manufacture and varnish manufacture.

10 One object of my invention is to provide a composition of matter in which the crystallization or partial separation of certain of the essential ingredients will be prevented. Another object of my invention is 15 to provide a method of combining the ingredients homogeneously, so that in the resulting composition they will stay permanently homogeneous. A further object of my invention is to provide a composition in 20 which the inflammability is reduced to an important extent below that of ordinary compositions containing cellulose nitrate. Yet another object is to produce a composition which may be made into permanently 25 transparent, strong and flexible sheets of film of desired thinness that are substantially waterproof, are unaffected by ordinary photographic fluids and possess the desired properties of a support for sensitive 30 photographic coatings. Still another object is to produce a composition which is capable of easy manipulation in the film making or varnish making arts; which will not injure or be injured by the substances with 35 which it is associated during manufacture, storage, or use. Further objects will hereinafter appear.

It is well known that pyroxylin compounds tend to burn with rapidity, so that 40 when present in the form of sheets or films, such as are used in motion picture projectors, for example, precautions against fire are advisedly taken. I have found that a composition with which the fire risk is lessened and one having the desirable quantities 45

hereinabove enumerated can be obtained by mixing or compounding cellulose nitrate with crystalline or waxy higher chlorin derivitives of the cyclic hydrocarbons  $C_{2n}H_{n+8}$  and their homologues, such as tri or 60 tetrachlor naphthalenes or anthracenes. Furthermore this compounding is preferably performed by mixing the ingredients with a solvent common to both, like methyl alcohol of the grade used in the pyroxylin 65 arts. If, however, the waxy body alone is thus compounded with the cellulose nitrate in serviceable amounts, it tends to separate out or crystallize on the surface of the varnish or film when the volatile common solvent evaporates, thus rendering it imperfect for some purposes, particularly impairing the transparency needed in the photographic art. I have discovered that this undesirable separation may be prevented by 70 incorporating phenyl esters, like triphenyl phosphate and its derivatives and homologues, into the compound along with the chlor body. Such phenyl esters are 75 peculiarly desirable as fixers of the chlor body, because they not only retain such body in its amorphous or colloidized state, but also tend to decrease the combustibility of the resulting composition, being themselves substantially non-combustible. When flexibility should be emphasized, as in photographic film, I also may add substances like the aliphatic alcohols of more than two carbon atoms,—for instance, fusel oil or the various butyl alcohols which have only 80 85 slight volatility.

The waxy chlor bodies which I employ are so substantially non-volatile that any loss under the conditions prevailing during the use and desired life of the film will not 90 make the latter unserviceable. As applied to my compounds, the term "non-inflammable" means, of course, only practical non-inflammability, the chlor bodies themselves not acting normally to propagate combustion but rather being strongly flame resisting. They impart this quality to a very useful degree to the composition in which I incorporate them. The following substance 95 may be mentioned as a typical example of the chlor body which I use. It is translucent and waxy with a somewhat crystalline appearance and consists of a mixture of higher chlorinated naphthalenes, chiefly tetrachlor naphthalenes. It has a boiling 100 105 110

range of 310° C. to 340° C. It is especially non-inflammable.

In carrying out one illustration of my invention I incorporate with 100 parts of cellulose nitrate 475 parts of methyl alcohol, 40 parts of fusel oil, 30 parts of triphenyl phosphate and 5 parts of the waxy chlor body mentioned hereinabove in the preceding paragraph. As before explained, 10 the fusel oil is optional but is preferable where enhanced flexibility is desired. In combining the ingredients, the cellulose nitrate and fusel oil are thoroughly mixed with the methyl alcohol while the triphenyl 15 phosphate and waxy chlor body are separately combined by means of a small portion of acetone, say 10 parts. This triphenyl phosphate-chlor body mixture is then thoroughly stirred into the cellulose 20 nitrate-fusel oil mixture to form a homogeneous solution or flowable mass, which may be filtered if desired. The pre-mixing of the triphenyl phosphate with the chlor body facilitates the introduction of the latter into the mixture and its continued presence keeps the chlor body from changing to the crystalline form or separating out.

This solution is sufficiently thick and viscous to be properly flowed during sheet 30 or film manufacture, the methyl alcohol volatilizing but not too rapidly to impair the product. The resulting film containing the non-volatilized ingredients is so flexible, smooth, transparent and uniform that it 35 may be used for any usual or preferred purpose. Due to its reduced inflammability, its fire risk is very much diminished. It is practically waterproof and is unaffected by ordinary photographic chemicals. The 40 chlor body, having the halogen in the ring or closed chain, is very stable, so that chlorin is not liberated in sufficient amounts to injure metal or other parts with which it comes in contact during manufacture and, 45 moreover, does not chemically re-act with or injure other bodies that it is associated with in the solution or film, even when the latter is coated with sensitive emulsion.

While I have herein disclosed certain 50 positions and processes by way of example, my invention is not limited to the proportions given therein, as my experiments indicate that the proportions may be widely varied from those given in order to adapt 55 the composition to particular uses. Furthermore equivalent substances may be substituted, such, for instance, as the solvent acetone in place of methyl alcohol.

Having thus described my invention, what 60 I claim as new and desire to secure by Letters Patent is:

1. A composition of matter comprising cellulose nitrate, a waxy higher chlorin derivative of the cyclic hydrocarbons  $C_{2n}H_{n+3}$ , 65 and their homologues and a non-inflammable

compound for preventing separation of said chlorin derivative.

2. A composition of matter comprising cellulose nitrate, a waxy higher chlorin derivative of the cyclic hydrocarbons  $C_{2n}H_{n+3}$  and their homologues, a non-inflammable compound for preventing separation of said chlorin derivative and a common solvent. 70

3. A composition of matter comprising cellulose nitrate, a waxy higher chlorin derivative of the cyclic hydrocarbons  $C_{2n}H_{n+3}$  and their homologues, a non-inflammable compound for preventing separation of said chlorin derivative and an organic body of slight volatility which enhances the 80 flexibility of the composition. 75

4. A composition of matter comprising cellulose nitrate, tetrachlor naphthalene and a phenyl ester for keeping said tetrachlor naphthalene in the colloidized state. 85

5. A composition of matter comprising cellulose nitrate, tetrachlor naphthalene and triphenyl phosphate.

6. A composition of matter comprising cellulose nitrate, tetrachlor naphthalene, a phenyl ester for keeping said tetrachlor naphthalene in the colloidized state and an organic body of slight volatility which enhances the flexibility of the composition. 90

7. A composition of matter comprising cellulose nitrate, tetrachlor naphthalene, triphenyl phosphate and fusel oil. 95

8. A composition of matter comprising cellulose nitrate, tetrachlor naphthalene, a phenyl ester for keeping said tetrachlor naphthalene in the colloidized state and a common solvent. 100

9. A composition of matter comprising cellulose nitrate, tetrachlor naphthalene, triphenyl phosphate, fusel oil and methyl alcohol. 105

10. A composition of matter comprising cellulose nitrate 100 parts, methyl alcohol 475 parts, fusel oil 40 parts, triphenyl phosphate 30 parts, a waxy chlorinated body consisting chiefly of tetrachlor naphthalene and boiling from 310° C. to 340° C. 5 parts and acetone 10 parts. 110

11. As an article of manufacture, a sheet of deposited or flowed cellulose nitrate containing a waxy higher chlorin derivative of the cyclic hydrocarbons  $C_{2n}H_{n+3}$  and their homologues and a non-inflammable compound for preventing separation of said chlorin derivative. 115

12. As an article of manufacture, a sheet of deposited or flowed cellulose nitrate containing tetrachlor naphthalene and a phenyl ester for keeping said tetrachlor naphthalene in the colloidized state. 120

13. As an article of manufacture, a sheet of deposited or flowed cellulose nitrate containing tetrachlor naphthalene and triphenyl phosphate.

14. As an article of manufacture, a sheet 130

of deposited or flowed cellulose nitrate containing tetrachlornaphthalene, triphenyl phosphate and fusel oil.

15. The process of making a composition of matter which comprises the step of combining tetrachlornaphthalene and triphenyl phosphate by the aid of a common solvent and then combining the resulting mixture with a solution containing cellulose nitrate.

16. The process of making a composition of matter which comprises first colloidizing tetrachlornaphthalene and triphenyl phosphate together and then combining the resulting mixture with a solution containing cellulose nitrate and fusel oil. 10

15  
Signed at Rochester, New York, this 23d day of December, 1919.

STEWART J. CARROLL.